

## UNITED STATES PATENT OFFICE

2,253,385

## STEEL

William E. Mahin, Murrysville, Pa., assignor to Westinghouse Electric & Manufacturing Company, East Pittsburgh, Pa., a corporation of Pennsylvania

No Drawing. Application January 29, 1941,  
Serial No. 376,420

5 Claims. (Cl. 75—128)

This invention relates to articles of manufacture and particularly to steel suitable for hot pressing and permanent molding operations.

Tool steel employed heretofore as dies for hot pressing and permanent molding operations where the tool is repeatedly heated at temperatures of more than 1000° F. have failed in a relatively short time by cracking, warping or washing. In general, it can be said that while the steels of previously known compositions have high hardness at elevated temperatures, they are not sufficiently resistant to oxidation, and particularly to intergranular oxidation, to have a long life. Intergranular oxidation results in development of points of stress concentration which cause surface cracking. Surface cracks grow inwardly and ultimately lead to failure of the die or mold.

Tool steels with high tungsten contents have long been known to possess very high red hardness, that is, high hardness at relatively high temperatures. Likewise steels with high chromium contents have been known to possess high resistance to oxidation at relatively high temperatures together with moderately high red hardness. The high tungsten steels have never been considered oxidation-resistant and therefore have usually been limited in use to applications where temperatures in service do not exceed a temperature of approximately 1200° F.

Contact surfaces of dies and molds used for hot pressing and molding or casting, particularly of non-ferrous metals and alloys probably reach temperatures well in excess of 1000° F. At these higher temperatures, ordinary tool steels containing high tungsten but relatively low chromium contents do not possess adequate oxidation resistance. On the other hand, previously known high chromium steels with relatively low contents of other hardening elements do not possess red hardness for most tool applications.

It is an object of this invention, therefore, to provide a steel having a high hardness at elevated temperatures, together with resistance to oxidation.

Another object of this invention is to provide a steel having a high tungsten and a high chromium content which will have a high hardness at elevated temperatures together with resistance to oxidation.

Other objects of this invention will become apparent from the following description and the appended claims.

It has been found in accordance with this invention that if tungsten and chromium are com-

bined in a steel in relatively high proportions, a steel is produced having a toughness, hardness and resistance to oxidation which renders it suitable for use as a die for hot pressing and permanent molding operations at repeated high temperatures.

The following table sets forth the broad ranges in percent by weight within which the several alloying elements may be present:

|             | Percent       |
|-------------|---------------|
| Carbon      | 0.05 to 0.50  |
| Manganese   | 0.15 to 3.00  |
| Silicon     | 0.20 to 1.00  |
| Chromium    | 8.00 to 20.00 |
| 15 Tungsten | 8.00 to 20.00 |
| Vanadium    | 0.10 to 4.00  |

the remainder being substantially all iron, together with such alloying impurities as are sometimes found in alloy steels.

A somewhat narrower range of percentages in which the several alloying elements may be present are as follows:

|             | Percent        |
|-------------|----------------|
| Carbon      | 0.05 to 0.30   |
| Manganese   | 0.15 to 0.50   |
| Silicon     | 0.20 to 0.50   |
| Chromium    | 11.00 to 15.00 |
| 25 Tungsten | 11.00 to 15.00 |
| Vanadium    | 0.10 to 1.00   |

the remainder being substantially all iron, together with such alloying impurities as are sometimes found in alloy steels.

Steels having the composition given in the foregoing tables are found to be satisfactory when formed into dies for hot pressing and permanent molding operations, and particularly such operations on hot non-ferrous metals and alloys. In order to give the steel certain of the characteristics desired in a die, the steel may be subjected to a heat treatment, preferably after having been formed to the predetermined shape of the die. Where desired, the finishing of machining operations may be applied to the die after the heat treatment.

The heat treatment may comprise quenching the steel in oil or air from a temperature between 2100° F. and 2350° F. and then subjecting it to a tempering treatment at a temperature between 1100° F. and 1300° F. for a sufficient period of time to develop its hardness. A preferred heat treatment is to quench the steel from a temperature between 2250° F. and 2300° F. and temper it at a temperature of about 1200° F.

In making the steel for forming the dies, it is

found that it is quite easy substantially to duplicate the composition of the tools. As examples of certain of the dies produced which have compositions within the ranges given hereinbefore, the following are listed:

|           | Percent | Percent | Percent | Percent | Percent |
|-----------|---------|---------|---------|---------|---------|
| Carbon    | .25     | .20     | .20     | .24     | .12     |
| Manganese | .25     | .16     | .27     | .28     | .25     |
| Silicon   | .25     | .21     | .36     | .38     | .25     |
| Chromium  | 12.00   | 12.13   | 12.62   | 12.50   | 12.00   |
| Tungsten  | 8.00    | 12.71   | 12.62   | 12.89   | 12.00   |
| Vanadium  | .50     | .46     | .43     | .43     | .50     |

it being understood that the remainder of the composition of each of the specific examples given is substantially all iron together with such alloying impurities as are sometimes found in alloy steels.

As previously stated, it is found that the high chromium and high tungsten constituents cooperate to impart high red hardness and high oxidation resistance to the finished product. The vanadium and silicon constituents function primarily as deoxidants in the making of the steel and the vanadium is thought to impart resistance in the steel against grain coarsening during the heat treatment of the alloy. The higher contents of vanadium may also assist in developing red hardness. The manganese is thought to impart forgeability characteristics to the alloy. For most of the applications embodied by this invention, the lower carbon contents as set forth are thought to develop adequate hardness and to aid in obtaining a steel having greater toughness than would be obtained with the higher carbon contents. However, it is not desired to be limited in application of the principles herein set forth to the lower carbon contents.

Dies formed from high chromium and high tungsten steel referred to hereinbefore are found to be resistant to oxidation, checking, warping and washing. These dies may have a useful life of from twelve to fifteen times the life of the dies formed from the conventional high tungsten, low chromium steels such as, for example, the 15% tungsten, 3% chromium, .50% carbon, and .50%

vanadium steel available on the market at the present time when subjected to operations entailing the repeated heatings at temperatures of over 1000° F. The high chromium, high tungsten steel dies of this invention are particularly useful in the hot pressing of copper parts and permanent molding of aluminum bronzes.

I claim as my invention:

1. A tool steel suitable for hot pressing and permanent molding operations formed from an alloy composed of 8% to 20% chromium, 8% to 20% tungsten, 0.10% to 4% vanadium, 0.20% to 1% silicon, 0.15% to 3% manganese, 0.05% to 0.5% carbon and the balance substantially all iron.

2. A tool steel suitable for hot pressing and permanent molding operations formed from an alloy composed of 11% to 15% chromium, 11% to 15% tungsten, 0.10% to 1% vanadium, 0.2% to 0.5% silicon, 0.15% to 0.5% manganese, 0.05% to 0.3% carbon and the balance substantially all iron.

3. A tool steel suitable for hot pressing and permanent molding operations formed from an alloy composed of about 12.62% chromium, about 12.62% tungsten, about 0.43% vanadium, about 0.36% silicon, about 0.27% manganese, about 0.20% carbon and the balance substantially all iron.

4. A tool steel suitable for hot pressing and permanent molding operations comprising an alloy composed of 8% to 20% chromium, 8% to 20% tungsten, 0.10% to 4% vanadium, 0.20% to 1% silicon, 0.15% to 3% manganese, 0.05% to 0.5% carbon, and the balance substantially all iron formed to a predetermined shape and heat treated to give high hardness, the steel being characterized in that it is resistant to oxidation.

5. A tool steel comprising an alloy of 8% to 20% chromium, 8% to 20% tungsten, 0.10% to 4% vanadium, 0.20% to 1% silicon, 0.15% to 3% manganese, 0.05% to 0.5% carbon and the balance substantially all iron which has been quenched from a temperature between 2100° F. and 2350° F. and tempered at a temperature between 1100° F. and 1300° F.

WILLIAM E. MAHIN.